

## UNITED STATES PATENT OFFICE

2,061,158

## METHOD OF TREATING PECTIN

Glenn H. Joseph, Corona, Calif., assignor to California Fruit Growers Exchange, Los Angeles, Calif., a corporation of California

No Drawing. Application April 10, 1934,  
Serial No. 719,893

22 Claims. (Cl. 99—132)

This invention relates to a method of treating previously extracted, solid pectin whereby certain fundamental and inherent characteristics of the pectin may be changed.

5 Pectin is utilized commercially in the manufacture of various products, and each trade requires that the pectin have certain uniform characteristics, although such requirements differ for different trades and uses. Certain uses require 10 a pectin with a uniformly slow setting rate, while a pectin with an unvarying rapid setting rate is required for other uses. Heretofore it has been difficult, if not impossible, for a pectin manufacturer to manufacture pectin with a predetermined 15 and uniform setting time or rate. Different source materials and extraction methods produce pectins with differing and generally uncontrollable setting characteristics. There is, therefore, a distinct need for some method whereby 20 the setting time or setting rate of pectin can be controlled or modified.

This invention is based upon the discovery that it is possible to alter, at will, one of the inherent, 25 intrinsic and fundamental characteristics of pectin, namely, its setting time, or its inherent ability to cause gelation to proceed in a jelly batch at a certain definite rate. By the method and means of this invention, the setting time of any previously extracted pectin may be changed 30 in the desired direction. The setting time of a pectin, as used herein, refers to that interval of time which elapses between the instant at which a jelly batch containing standard proportions of sugar, acid, pectin and total solids is formed and 35 that at which gelation or jellification into a coherent mass can be observed.

Generally stated, the method comprises contacting the pectin with a reagent adapted to materially alter the intrinsic setting time of said 40 previously extracted pectin, and maintaining the reagent in contact with the pectin for a time and at a temperature insufficient to destroy the gelation characteristics of the pectin or materially affect the texture of the gel which may subsequently be formed from such treated pectin.

The treating reagent may be either liquid or gaseous, aqueous or anhydrous. The preferred reagent is an acid, an acidic, or an acid forming substance. For convenience in handling and application of the reagent, a liquid may be used as a carrier. The liquid medium should not act as a solvent or dispersing medium for the solid pectin being treated, and preferably the medium or carrier should not interact chemically with the 55 acid used under the conditions prevailing dur-

ing treatment. An acidified alcohol illustrates a desirable treating agent.

An object of the invention, therefore, is to disclose and provide a method of altering the setting time of a previously extracted pectin.

Another object is to disclose and provide a method of treating previously extracted pectin in various degrees of purity for the purpose of altering, and particularly retarding, the setting rate or time of the pectin.

A further object is to provide a method whereby it is possible to alter the characteristic setting time of a pectin to any desired definite and predetermined value.

Another object of the invention is to provide 15 a method and means for treating pectin with an acid reagent in the presence of a relatively non-dispersing organic liquid for the purpose of retarding the setting rate or increasing the setting time of a previously extracted pectin.

Other objects and advantages of the invention 20 will appear more fully and at large hereinafter.

It is to be understood that this invention is directed to the treatment of pectin in solid form and particularly to the treatment of a pectin 25 which has been previously extracted from a cellulosic source material. Various methods of extraction are known and need not be described herein. In such previously known methods, the pectin is precipitated from the extracts with 30 alcohol, by salting out or by the so-called aluminum precipitation process disclosed in patent No. 1,497,884.

It has been determined that the process of 35 this invention is applicable to pectins extracted from any source, such as, for example, citrus peel, apple pomace, etc. Moreover, the process does not appear to be influenced by the method of extraction, precipitation or purification used prior to the application of the process of this invention. The solid, preferably finely divided, pectin capable of being treated in accordance 40 with this invention may be either of a technical grade or of a more extensively purified grade. It may contain appreciable quantities of water 45 or it may be substantially dry.

As has been stated hereinbefore, the method 50 of the invention contemplates contact of a previously extracted solid pectin with a treating agent adapted to materially alter the intrinsic setting time of the pectin. The preferred process is carried out by contacting the pectin with an acidified liquid medium. In order to illustrate the process and results attained thereby, the following examples are given. In each of the fol- 55

lowing tests, 20 grams of dry pectin were contacted with 100 ml. of organic liquid to which there was added 10 ml. or 10 normal hydrochloric acid. The pectin was maintained in contact with the treating agent for a period of 24 hours at a temperature of 25° C. The pectin before treatment was found to set to a jelly under standard conditions of sugar and acid in 100 seconds (1.66 minute). The effect of various treating liquids upon the setting time of the pectin under these conditions were observed to be as follows:

| 15 | Liquid medium used              | Time of set |
|----|---------------------------------|-------------|
| 20 | Methyl alcohol (90%)            | 2.5         |
|    | Ethyl alcohol (80%)             | 8           |
|    | Isopropyl alcohol (90%)         | 13          |
|    | Tertiary butyl alcohol (80-85%) | 20          |
|    | Methyl ethyl ketone (100%)      | 25          |
|    | Acetone (100%)                  | 32          |

It is to be remembered that in each instance 10 ml. of 10 N. hydrochloric acid was added to 100 ml. of the organic medium. The percentages following the name of the liquid used are approximate for the concentration of the liquid before adding acid and pectin.

30 Dilution of the organic liquid used as a carrier for the acid influences the rapidity with which the setting time of the pectin is altered within a given contacting period. The effect of various ethyl alcohol—water mixtures (containing HCL 35 in the same proportions as that given hereinabove) on the setting time of the pectin is shown in the following table:

| 40  | ML liquid used                       |  | Set in minutes |
|-----|--------------------------------------|--|----------------|
| 45  | 95% C <sub>2</sub> H <sub>5</sub> OH |  |                |
|     | Water                                |  |                |
| 100 | None                                 |  | 4.75           |
| 85  | 15                                   |  | 9.5            |
| 65  | 35                                   |  | 15             |

In the above test, 10 ml. of 10 N. hydrochloric acid was added to the liquid and 20 grams of pectin brought into contact therewith and maintained in such contact for a period of about 43 hours at about 25° C. The dilution of the ethyl alcohol retards the set more energetically.

55 Absolute methyl alcohol when used as a carrier for the acid appears to accelerate the set instead of retarding the setting time. Upon dilution, methyl alcohol-acid mixtures retard or prolong the setting time. When acetone is diluted, on the other hand, it appears to lose some of its great ability to allow retardation of the setting time by the acid carried thereby. Although 100% acetone prolongs the setting time to 28 minutes when pectin having an original setting time of 1.66 minutes is treated with a mixture consisting of 100 ml. of acetone and 10 ml. of 10 N. hydrochloric acid for 12 hours at 25° C., a set of only 8 minutes is obtained when the treating liquid consists of 75 ml. acetone, 25 ml. water and 10 ml. of 10 N. hydrochloric acid.

Attention is called to the fact that after the setting rate of a pectin has been retarded by treatment with acid as here described, the setting rate can subsequently be accelerated (setting time shortened) by treatment with acid in

the presence of methyl alcohol. The setting time of a pectin can thus be repeatedly altered, as desired.

The treating agent should contain an acid or acidic component. When organic liquids are used as media for the acidic components, any of the mineral acids may be used whenever the organic liquid is a solvent therefor. Although sulfuric, sulfurous phosphoric and nitric acids are suitable, hydrochloric acid is the preferred acid. Organic acids such as lactic may also be used. When pectin is contacted with an aqueous acid solution in accordance with this invention, its setting time is altered (generally lengthened or prolonged) but due to imbibition of water, the pectin is more difficultly handled. As an illustration, when pectin is allowed to remain in contact with 85% lactic acid, a plastic mass is obtained which has to be hardened in 90% alcohol and ground.

20 The reagent used in obtaining the desired alteration in setting time of pectin may be anhydrous. The treating agent may comprise an acidic substance, such as chlorine, hydrogen sulfide, sulfur dioxide or sulfur trioxide. Pectin containing about 8% to 10% of moisture may be contacted with any of these acidic gases and an alteration in setting time obtained. Dry hydrogen chloride gas may also be used, either alone or dissolved in alcohol, benzol, or the like. An acidic material such as acid methyl sulfate, 25 may be used without any additional carrier.

It appears that any acid or acid radical may be employed, provided it is of sufficient activity and has no destructive action upon any of the constituents of the mixture. The more active acids uniformly produce retardation of the set in a shorter treating time than less active acids. The concentration of the acid used may also vary over a very wide range, for example, from 0.5% to as high as 25% HCl, the concentration of acid used being influenced by time and temperature conditions which it is desired to use. The higher the concentration of the acid, the shorter the treating time. With solutions containing high concentrations of acid, a treating time of only a few minutes may be sufficient. The use of very high concentrations of acid is not recommended, however, as some degradation of the pectin and a loss in jelly strength or jelly units may result.

40 The preferred organic liquids used as media contain the methyl radical, the acetyl radical or a saturated alkyl group. Specific examples of such liquids are methyl alcohol, ethyl alcohol, normal propyl alcohol, isopropyl alcohol, normal butyl alcohol, isobutyl alcohol, secondary butyl alcohol, tertiary butyl alcohol, amyl alcohol, isoamyl alcohol, ethyl ether, acetone, methyl ethyl ketone, acetyl chloride, ethyl acetate, acid 45 methyl sulfate, etc.

Among other liquids which may be used are aliphatic and aromatic hydrocarbons and their derivatives, the preferred liquids being the simpler aliphatic hydrocarbon derivatives such as alcohols, ketones, aldehydes, amines and ethers and the aromatics of low molecular weight, such as benzol. Air and gases or vapors which do not chemically react with the treating reagent to any substantial or detrimental degree are 50 fluid carriers coming within this invention.

Various organic liquids may be used as a carrier for the treating reagent. In general, the liquid media should not exert any appreciable solvent or dispersing effect upon the solid pectin.

because of the mechanical difficulties involved in handling mixtures of liquid with solid pectin, when the pectin swells excessively. Although the organic liquids (when miscible with water, as 5 diethylene glycol, for example) may be diluted with water, the relative proportion of water should not be increased to such a point that any excessive hydration and/or agglutination of the pectin particles takes place. Although dilution 10 of ethyl alcohol appears to increase the rate at which the setting time of the pectin is retarded, it is not ordinarily desirable to reduce the proportion of ethyl alcohol below about 45% of the total liquid, as further dilution gives rise 15 to mechanical difficulties incident to the swelling and hydration of the pectin particles.

The conditions of temperature, time and acid concentration affect the rapidity or the extent to which the setting time of the pectin is altered. When higher temperatures are used, the 20 time of contact may be shortened or a solution of lower acid concentration may be used to produce a desired effect. The fineness of division of the solid pectin being treated plays but a 25 secondary part. It is not necessary that the solid pectin be finely divided. Relatively coarse pectin in the form of flakes or in the fibrous condition which it assumes upon precipitation with alcohol, may be treated just as effectively as a 30 solid pectin disintegrated sufficiently to pass through a 60 mesh screen. When treating solutions of higher acid concentration are used, better results are obtained by having the pectin in a finely divided condition so as to pass through 35 a 40, 80 or 100 mesh.

As a result of some processes of extracting pectin, the pectin particles contain residual acid. Usually the pectin is washed repeatedly with alcohol or other solvent in which the pectin is difficultly soluble or insoluble (such as a solution 40 of a salt of a strong base and a weak acid) in order to controllably reduce the acid and other possible impurities. In accordance with this invention, however, the acid-containing pectin resulting from such processes may be stored for an appreciable time in a substantially dry condition (from about 2% to 10% H<sub>2</sub>O) or with the addition of but enough moisture to dampen the pectin, and thereby permit the setting time of 45 the pectin to be altered or prolonged.

After a previously extracted solid pectin has been treated in the manner described hereinabove, it may be washed or rinsed with fresh or neutral alcohol or other suitable solvent, and 50 then dried. The solvent used may contain a buffer salt, such as sodium citrate or sodium carbonate, or an alkali. The removal of residual acidity stabilizes the pectin and stops further alteration in setting time. After washing, 55 the pectin may be dried in any suitable manner and if necessary reduced to the desired state of division. Whenever the ultimate use of the pectin is facilitated thereby, the pectin may be standardized as to jelly grade or admixed with 60 suitable quantities of acid or acid-forming materials, additional buffer salts, sugar, and similar materials.

It will be evident from the description given hereinabove that a process has been disclosed 70 which permits the manufacturer, dealer or user of pectin to alter at will the setting time of this substance. Although as stated hereinabove, the primary object attained by the method is the alteration in setting or gelation time of the 75 pectin, other advantageous results are obtained

at the same time. Even though some mechanical losses may be encountered in the practice of the method, for example, an improvement in the actual grade of the pectin is obtained when the process is carried out under optimum conditions, so that the jelly unit yield is over 100%. The pectin treated in accordance with this invention is generally lighter in color than the original solid pectin, has a lower ash content, and there is some indication that the treated 10 pectin is ground more readily than the pectin not so treated.

Although specific materials have been mentioned hereinabove as suitable reagents for use in the process of this invention, they have been 15 set forth for purposes of illustration only and the invention is not limited thereto. All changes, modifications and equipments coming within the scope of the appended claims are embraced 20 thereby.

I claim:

1. A method of treating pectin which comprises contacting solid, previously extracted pectin in the form of discrete particles with an acidic reagent adapted to materially alter the 25 intrinsic setting time of the pectin, the pectin being maintained in contact with the reagent for a period of time and at a temperature insufficient to destroy the gelation characteristics of the pectin but sufficient to materially alter the 30 intrinsic setting time hereof.

2. A method as defined in claim 1, in which the reagent comprises a non-dispersing liquid medium incapable of dissolving the pectin to any appreciable extent, and an acid.

3. A method as defined in claim 1, in which the reagent comprises an acid.

4. A method of treating pectin as defined in claim 1, in which the reagent is an acidic gas from the group consisting of hydrogen chloride, 40 chlorine, hydrogen sulfide, sulfur dioxide and sulfur trioxide.

5. A method of treating pectin as defined in claim 1, in which the reagent comprises an organic liquid, and an acidic component.

6. A method of treating pectin as defined in claim 1, in which the reagent comprises a water-miscible organic liquid, and an acid.

7. A method of treating pectin as defined in claim 1, in which the reagent comprises a water-miscible organic liquid, an acid and water in quantity insufficient to exert a material solvent action upon the pectin.

8. A method of treating pectin as defined in claim 1, in which the reagent comprises an organic liquid containing a methyl radical, and an acid.

9. A method of treating pectin as defined in claim 1, in which the reagent comprises an organic liquid containing the acetyl radical, and 60 an acid.

10. A method of treating pectin as defined in claim 1, in which the reagent comprises an organic liquid from the group consisting of the alcohols, ketones, aldehydes, glycols and benzol 65 containing the methyl radical, the acetyl radical, or a saturated alkyl group, and an acid.

11. A method of treating pectin as defined in claim 1, in which the reagent is maintained in substantial contact with the pectin for a period 70 of time of from 1 to 48 hours.

12. A method as defined in claim 1, in which the reagent comprises a non-dispersing liquid medium incapable of dissolving the pectin to any appreciable extent, and an acid, the reagent 75

- being in quantity sufficient to completely moisten the surfaces of the pectin particles.
13. A method of treating pectin whereby the setting time thereof is altered, which comprises 5 contacting previously extracted solid pectin in the form of discrete particles with a carrier having substantially no solvent or dispersing action on the pectin, said carrier containing an acid radical, and maintaining the carrier and its 10 acid radical in contact with the pectin for a time sufficient to materially alter the setting time of the pectin.
14. A method as defined in claim 13 in which the pectin is washed after contact to diminish 15 residual acidity thereof.
15. A method of treating pectin whereby the setting time thereof is altered, comprising contacting solid pectin with an acidic reagent and maintaining such contact for a time sufficient 20 to materially alter the setting time of the pectin but insufficient to destroy the gelatin characteristics of the pectin, then separating the pectin from the acidic reagent, and washing the pectin to diminish residual acidity thereof.
- 25 16. A method of treating pectin as defined in claim 1 in which the reagent comprises an organic liquid containing a saturated alkyl group, and an acid.
17. A method of treating a previously extracted solid pectin which comprises contacting 30
- pectin in the form of discrete particles with an aqueous liquid containing more than 45% of ethyl alcohol and an acidic component, for a length of time sufficient to alter the setting time of the pectin. 5
18. A method of treating a previously extracted solid pectin which comprises contacting pectin in the form of discrete particles with methyl alcohol containing an acidic component, for a length of time sufficient to alter the setting time of the pectin. 10
19. A method of treating pectin as defined in claim 1 in which the reagent comprises an organic liquid incapable of dissolving the pectin to any appreciable extent. 15
20. A method of treating pectin as defined in claim 1 in which the reagent comprises a water miscible organic liquid incapable of dissolving the pectin to any appreciable extent. 15
21. A method of treating pectin as defined in claim 1 in which the reagent comprises a water miscible organic liquid incapable of dissolving the pectin to any appreciable extent, and an acid. 20
22. A method of treating pectin as defined in claim 1 in which the reagent comprises an organic liquid incapable of dissolving the pectin to any appreciable extent, and an acid. 25

GLENN H. JOSEPH. 30

CERTIFICATE OF CORRECTION.

Patent No. 2,061,158.

November 17, 1936.

GLENN H. JOSEPH.

It is hereby certified that error appears in the printed specification of the above numbered patent requiring correction as follows: Page 2, first column, line 3, for the word "or" read of; page 3, second column, line 71, claim 11, after "from" insert about; and that the said Letters Patent should be read with these corrections therein that the same may conform to the record of the case in the Patent Office.

Signed and sealed this 16th day of February, A. D. 1937.

(Seal)

Henry Van Arsdale  
Acting Commissioner of Patents.

- being in quantity sufficient to completely moisten the surfaces of the pectin particles.
13. A method of treating pectin whereby the setting time thereof is altered, which comprises 5 contacting previously extracted solid pectin in the form of discrete particles with a carrier having substantially no solvent or dispersing action on the pectin, said carrier containing an acid radical, and maintaining the carrier and its 10 acid radical in contact with the pectin for a time sufficient to materially alter the setting time of the pectin.
14. A method as defined in claim 13 in which the pectin is washed after contact to diminish 15 residual acidity thereof.
15. A method of treating pectin whereby the setting time thereof is altered, comprising contacting solid pectin with an acidic reagent and maintaining such contact for a time sufficient 20 to materially alter the setting time of the pectin but insufficient to destroy the gelatin characteristics of the pectin, then separating the pectin from the acidic reagent, and washing the pectin to diminish residual acidity thereof.
- 25 16. A method of treating pectin as defined in claim 1 in which the reagent comprises an organic liquid containing a saturated alkyl group, and an acid.
17. A method of treating a previously extracted solid pectin which comprises contacting 30
- pectin in the form of discrete particles with an aqueous liquid containing more than 45% of ethyl alcohol and an acidic component, for a length of time sufficient to alter the setting time of the pectin. 5
18. A method of treating a previously extracted solid pectin which comprises contacting pectin in the form of discrete particles with methyl alcohol containing an acidic component, for a length of time sufficient to alter the setting time of the pectin. 10
19. A method of treating pectin as defined in claim 1 in which the reagent comprises an organic liquid incapable of dissolving the pectin to any appreciable extent. 15
20. A method of treating pectin as defined in claim 1 in which the reagent comprises a water miscible organic liquid incapable of dissolving the pectin to any appreciable extent. 15
21. A method of treating pectin as defined in claim 1 in which the reagent comprises a water miscible organic liquid incapable of dissolving the pectin to any appreciable extent, and an acid. 20
22. A method of treating pectin as defined in claim 1 in which the reagent comprises an organic liquid incapable of dissolving the pectin to any appreciable extent, and an acid. 25

GLENN H. JOSEPH. 30

CERTIFICATE OF CORRECTION.

Patent No. 2,061,158.

November 17, 1936.

GLENN H. JOSEPH.

It is hereby certified that error appears in the printed specification of the above numbered patent requiring correction as follows: Page 2, first column, line 3, for the word "or" read of; page 3, second column, line 71, claim 11, after "from" insert about; and that the said Letters Patent should be read with these corrections therein that the same may conform to the record of the case in the Patent Office.

Signed and sealed this 16th day of February, A. D. 1937.

(Seal)

Henry Van Arsdale  
Acting Commissioner of Patents.

CERTIFICATE OF CORRECTION.

Patent No. 2,061,158.

November 17, 1936.

GLENN H. JOSEPH.

It is hereby certified that error appears in the printed specification of the above numbered patent requiring correction as follows: Page 2, first column, line 3, for the word "or" read of; page 3, second column, line 71, claim 11, after "from" insert about; and that the said Letters Patent should be read with these corrections therein that the same may conform to the record of the case in the Patent Office.

Signed and sealed this 16th day of February, A. D. 1937.

Henry Van Arsdale  
Acting Commissioner of Patents.

(Seal)